

## UNITED STATES PATENT OFFICE

STEWART J. CARROLL, OF ROCHESTER, NEW YORK, ASSIGNOR TO EASTMAN KODAK COMPANY, OF ROCHESTER, NEW YORK, A CORPORATION OF NEW YORK

## CELLULOSE-ETHER FILM AND COMPOSITION FOR MAKING THE SAME

No Drawing.

Application filed August 9, 1926. Serial No. 128,338.

This invention relates to compositions of matter in which cellulose ethers, such as water-insoluble ethyl cellulose, are combined or mixed with other substances which impart 5 not only low inflammability, but likewise give compositions the other properties of which are also highly advantageous in the plastic and analogous arts, such, for instance, as the film or varnish arts.

10 One object of the invention is to provide cellulose ether films having not only all of the ordinary desirable qualities of films for photographic purposes, but also having unusually low inflammability and extremely high resistance to deterioration by 15 heat. Another object of the invention is to provide permanently transparent, strong, flexible sheets or films of desired thinness, which are substantially waterproof, are 20 unaffected by ordinary photographic fluids, are substantially colorless, are substantially without harmful action upon light-sensitive photographic coatings, are of low inflammability and highly resistant to prolonged heating. Another object of the 25 invention is to provide compositions capable of easy manipulation in film making, varnish making, or allied plastic arts. Another object is to provide compositions which will not injure or be injured by the substances or 30 surfaces with which they are associated during manufacture, storage or use. Other objects will hereinafter appear.

In U. S. Patent No. 1,188,376 Lilienfeld, 35 June 20th, 1916, there are disclosed a series of alkyl ethers of cellulose. Certain of these are particularly insoluble in water, and the present invention finds its chief value in connection with ethers having this property, such as water-insoluble ethyl cellulose, films of which have small shrinkage characteristics, after treatment in photographic baths. In U. S. Patent No. 1,583,709, Webb, May 4th, 1926, there are disclosed films of such cellulose ethers in which the ordinary desirable qualities of photographic film base are combined with resistance to prolonged heating, this result being brought about by maintaining an alkalinity in excess of pH 7. It is desirable that such films, especially motion pic-

ture films, be capable of withstanding heating without becoming brittle. Whether or not films will possess this property can be foretold with practical accuracy by testing samples, say by heating them for weeks and even months at a continuous temperature of 65° C. Films which remain usefully flexible after such a severe test are capable of withstanding the conditions met with in use.

I have found that these qualities of the 60 films may be maintained and yet the inflammability greatly lowered by incorporating in such films and in the compositions out of which they are made, one or more of the brom-nucleo (mono and polybrom) substitution 65 products of naphthalene, anthracene and their homologues. The isomers resulting from different positions of the brom atoms on the rings, are all usable. On account of its relative cheapness and simplicity of manufacture, I prefer alpha bromnaphthalene. All of these substances, when mixed into the 70 film-making compositions, should be free from free bromine and free hydrobromic acid. Otherwise they will cause sufficient discoloration to make the film undesirable for photographic purposes, will cause deterioration of any photographic emulsions placed upon the films, and will destroy the alkalinity 75 upon which the resistance of the film to prolonged heating depends.

But I have found, as stated above, that if the brominated products are initially purified from free bromine and free hydrobromic acid and are incorporated in films having an 80 alkalinity greater than pH 7, there is no acidity in the film-making solution, nor in the film, nor does this condition develop during the normal storage of the solution or during the normal useful life of the film.

I shall now give one example of my invention by way of illustration, but it will be understood that the invention is not limited to these details, except as indicated in the appended claims. 100 parts by weight of 85 water-insoluble ethyl cellulose containing sufficient alkali, say by undergoing the treatment given in lines 78 to 92 of page 1 in the above cited Webb patent, are dissolved along with 5 to 50 (say 20 parts) of alpha 90

55

65

70

75

80

85

90

95

100

bromnaphthalene in 300 to 500 parts of a volatile common solvent. The latter may usefully comprise a mixture of methyl acetate and methyl alcohol, the weight of the methyl acetate being approximately nine times the weight of the methyl alcohol. Of course, the ingredients of the solvent are of sufficient purity to avoid acidifying the composition. This composition is suitable for spreading upon a film-forming surface in a coating, from which the volatile solvent evaporates sufficiently to leave a transparent, flexible sheet, which is stripped off and otherwise treated in a manner well known to those skilled in this art. In place of the alpha bromnaphthalene, an equal number of parts by weight can be substituted of any one of the brominated bodies mentioned hereinabove, or mixtures of them. By reason of the fact that these brominated products are of the nucleo type, having the bromine atoms directly bonded to the ring of carbon atoms, they are particularly stable.

The ingredients in the film-forming composition are thoroughly mixed and may be filtered if desired. When more flowable solutions are desired, or when the compositions are to be employed as lacquers, the volatile solvent may be increased until the desired viscosity is obtained, or volatile liquids, such as benzol, alcohol, and the like may be added to the thinner. Along with the ingredients mentioned above, I may add one or more supplementary organic bodies of only slight volatility which enhance the flexibility of the compositions and regulate the preparation of film therefrom; but such bodies are not essential. Examples of them are amyl or butyl acetate, the various amyl alcohols, the various butyl alcohols, and mixtures of them. Of course, these ingredients are also sufficiently pure to be non-acid.

Films prepared from the hereinabove described compositions are flexible, smooth, transparent, strong, substantially colorless, substantially waterproof, are unaffected by ordinary photographic baths, and in addition, combine unexpectedly low inflammability with high resistance against brittleness upon prolonged heating at 65° C., or equivalent conditions in actual use. The amount of alkali in the films is, of course, insufficient to impair their transparency.

Having thus described my invention, what I claim as new and desire to secure by Letters Patent is:

1. A flowable film-forming composition comprising a water-insoluble cellulose ether, a brom-nucleo substitution product of the class comprising naphthalene, anthracene, and their homologues, which product is substantially free from uncombined bromine and hydrobromic acid, and a solvent common to said ingredients, said composition being stabilized by the presence therein of inor-

ganic alkali which creates an alkalinity in the composition in excess of pH 7 the specified ingredients being present in such proportions as to produce a transparent, colorless flexible film.

2. A flowable film-forming composition comprising 100 parts by weight of water-insoluble ethyl cellulose, 5 to 50 parts of alpha bromnaphthalene substantially free from uncombined bromine and hydrobromic acid, and more than 300 parts of a volatile common solvent, said composition comprising sufficient inorganic alkali to give it an alkalinity in excess of pH 7 the specified ingredients being present in such proportions as to produce a transparent, colorless, flexible film.

3. As an article of manufacture a flexible, transparent, colorless film comprising colloidized water-insoluble cellulose ether and a brom-nucleo substitution product of the class comprising naphthalene, anthracene, and their homologues, said product being substantially free from uncombined bromine and hydrobromic acid, said film having distributed therein sufficient inorganic alkali to give the film an alkalinity in excess of pH 7.

4. As an article of manufacture, a flexible, transparent, colorless film comprising colloidized water-insoluble ethyl cellulose and alpha bromnaphthalene free from uncombined bromine and hydrobromic acid, said film having uniformly distributed therein sufficient inorganic alkali to give the film an alkalinity in excess of pH 7, the amount of alkali being insufficient to impair the transparency of the film.

Signed at Rochester, New York this 29th day of July, 1926.

STEWART J. CARROLL.

105

110

115

120

125

130